

July 24, 1928.

1,678,145

M. J. KELLY

ELECTRON DISCHARGE DEVICE

Filed July 8, 1924



Inventor:  
Mervin J. Kelly,  
by *Edward A. Adams, Atty*

## UNITED STATES PATENT OFFICE.

MERVIN J. KELLY, OF NEW YORK, N. Y., ASSIGNOR TO WESTERN ELECTRIC COMPANY, INCORPORATED, OF NEW YORK, N. Y., A CORPORATION OF NEW YORK.

## ELECTRON-DISCHARGE DEVICE.

Application filed July 8, 1924. Serial No. 724,754.

This invention relates to electron discharge devices and has for an object a low impedance device of this character having a high amplification factor in which the electron emitting element may be energized by alternating current.

This object is attained by utilizing as a cathode a thermionically active member having a large active surface and energizing this member by means of a heating element separate therefrom. For the thermionically active member there is provided a metallic cylinder coated with alkaline earth oxides. Associated with this cylinder is an electric resistance element by means of which heat is applied to the cylinder to activate the oxides. A control electrode surrounds the cathode and comprises a helical wire grid. The surface of the grid wire is oxidized in order to prevent its becoming thermionically active due to the deposition of a layer of alkaline earth oxides vaporized thereon from the cathode. Surrounding the grid and cathode is a cylindrical anode, which is composed of decarbonized nickel to prevent the reduction of the oxide coating of the grid during the evacuation of the tube by carbon supplied from the anode.

All the elements are supported at one end within the enclosing vessel of the device from the stem thereof by metallic means and the free ends of the elements are tied with insulating material to form a rigid unitary structure.

By virtue of the geometric arrangement of the electrodes and the large active cathode surface, the impedance of this device is very low and its space current correspondingly high. As a result the amplification factor can be made much higher for the same output impedance than electron discharge devices of corresponding size having filamentary cathodes. Moreover, the cathode has the same potential throughout its surface and the voltage drop between it and the anode is, therefore, uniform. Alternating current may be supplied to the heating element to activate the cathode without introducing any disturbances into the operation of the tube, since there is no current flow in the cathode itself.

Referring now to the drawings, Fig. 1 discloses an electron discharge device constructed in accordance with the invention. Fig. 2 discloses the heating unit and Fig. 3

discloses the heating unit combined with the cathode.

The enclosing vessel 10 of the device is provided with an inwardly projecting stem 11. A pair of rods 12 are sealed in the end of the stem 11 and extend longitudinally of the tube, their ends being seated in a block 13 of insulating material, preferably of the material commercially known as "lavite." A rod 14 is also sealed in the stem midway between the rods 12 and extends through the block 13, its free end being slideable in the block. Supported on the rod 14 is a core or spool 15 of refractory material having a high thermal conductivity and a low electrical conductivity. As shown in Fig. 2, a filament 16, preferably of tungsten wire, is wound around the spool. The wire 16 is covered with a coating 17 of alundum cement. Surrounding the spool 15 and supported thereby is a metallic cylinder 18, preferably of nickel, which is coated with a thermionically active material. This coating preferably is composed of a mixture of strontium and barium oxides. One end of the filament 16 is welded to the rod 14 at 19 and the other end is connected to the leading-in wire 20. A leading-in wire 21 is attached to the opposite end of the rod 14 whereby heating current may be supplied to the filament 16. A leading-in wire 22 is provided for the cathode 18.

Surrounding the cathode is a grid or control electrode 23 which comprises a pair of longitudinal rods or wires 24 between which is helically wound a lateral wire 25. Both the rods 24 and the wire 25 are composed of nickel or an alloy thereof which has been oxidized to form on the surface a coating of nickel oxide. One of the rods 24 is welded to a leading-in wire 26 which also serves as a supporting wire, and the opposite end of this rod together with the corresponding end of the other rod 24 is slidably mounted in the insulating block 13.

The anode 27 comprises a metallic cylinder supported between the rods 12 by means of the members 28 and surrounds the other elements. This cylinder is composed of a metal, preferably nickel, from which all carbon has been removed for a considerable depth from the surface. A leading-in wire 29 for the anode is joined to the end of one of the rods 12.

The grid electrode is provided with a coat-

ing of nickel oxide to prevent it becoming thermionically active by the deposition thereon of alkaline earth oxides volatilized from the cathode, the temperature of the grid during the operation of the device being high enough to activate these oxides. A nickel oxide layer interposed between the nickel surface and the alkaline earth oxides makes a thermionically inactive surface at any temperature. Decarbonized nickel is used as the material of the anode to prevent reduction of the nickel oxide coating of the grid during the evacuation of the tube. If the carbon is not removed from the anode it reacts with water vapor and oxygen within the tube to form carbon monoxide. Carbon monoxide, if present in the tube, reduces the oxide coating on the grid to give a clean grid surface. Depositions on the clean grid surface of alkaline earth oxides from the cathode render these portions of the grid thermionically active. The water vapor above mentioned comes from the glass envelope of the device and from the electrodes. The oxygen comes from the same parts and probably from the reduction of the alkaline earth oxide coating on the cathode. There is usually so much water vapor and oxygen within the containing vessel of the device that sufficient carbon monoxide is formed to reduce the oxide coating of the grid to such an extent that enough alkaline earth oxides are deposited on bare spots thereon to render the grid so active thermionically as to prevent proper operation of the device. Also, the long continued reaction between the carbon and water vapor and oxygen destroys to a large extent the activity of the cathode. However, the use of an anode of decarbonized nickel prevents the formation of carbon gases and permits the device to be evacuated quickly and without reduction of the nickel oxide coating of the grid.

Because of the comparatively large surface area of the cathode, the space current between it and the anode is very large and the device has a high amplification factor. It is, therefore, possible to obtain greater degrees of amplification with corresponding plate voltages than has heretofore been possible.

It is, of course, understood that various modifications may be made in the structure and arrangement of the various elements of the device above described without in any way departing from the spirit of the invention, as set forth in the appended claims.

The invention claimed is:

1. An electron discharge device comprising an enclosing vessel having a re-entrant stem, a pair of rods extending from said stem, a block of insulating material joining the free ends of said rods, another rod having one end sealed in said stem and the other end slidably mounted in said insulating

block, a heating element insulatingly supported on said rod, a metallic cylinder surrounding said heating element and insulatingly supported thereby, a grid element supported from said stem and said insulating block, and a cylindrical anode surrounding said other elements and supported from said first two rods. 70

2. An electron discharge device comprising a metallic rod, a spool of refractory material carried thereby, a metallic cylinder supported by said spool, said cylinder having a thermionically active surface, and an electric resistance embedded in said spool. 75

3. An electron discharge device comprising an enclosing vessel having a stem, a metallic rod sealed in said stem, a leading-in wire for said rod, a spool of refractory material carried by said rod, a cylinder having a thermionically active surface supported by said spool, a resistance element embedded in said spool and having one end connected to said rod, and a leading-in wire connected to the opposite end of said resistance element. 80

4. An electron discharge device comprising a vessel having a stem, a plurality of rods sealed in said stem, a block of insulating material connecting the free ends of said rods, the end of one rod being slidably in said block, a thermionically active member supported by said last named rod, a metallic cylinder supported by said other rods, and leading-in wires connected to certain of said rods. 95

5. An electron discharge device comprising an enclosing vessel having a stem, a pair of rods sealed in said stem, a leading-in wire for one of said rods, a block of insulating material joining together the free ends of said rods, another rod sealed in said stem and having its free end slidably mounted in said insulating block, a leading-in wire for said rod, an electrical heating unit carried by said rod and having one end connected thereto, a leading-in wire for the other end of said heating unit, a thermionically active cylinder supported by said heating unit, a grid electrode surrounding said cylinder and being slidably supported by said block of insulating material, and a cylindrical anode surrounding said grid and supported by said first two named rods. 105

6. A cathode for electron discharge devices comprising an electrical conductor, a spool of electrically non-conductive material having high thermal conductivity carried by said conductor, a filamentary conductor wound on said spool and having one end connected to said first conductor, a layer of electrically non-conductive cement covering said filamentary conductor, and a thermionically active cylinder surrounding said spool and supported thereby. 115

7. An electron discharge device comprising 120

ing an enclosing vessel having a stem, a pair of metallic rods sealed in said stem and having their free ends connected by a block of insulating material, a cylindrical anode supported by said metallic rods, a thermionically active member supported by a rod sealed in said stem, a grid electrode supported by

a metallic member sealed in said stem, said grid electrode and said last named rod being slidably connected to said insulating block. 10

In witness whereof, I hereunto subscribe my name this 2 day of July A. D., 1924.

MERVIN J. KELLY.